# EUROPEAN PATENT SPECIFICATION

(11) **EP 0 934 127 B1**
(45) Date of publication and mention of the grant of the patent: **26.09.2001**
(21) Application number: 97913758.5
(22) Date of filing: 24.10.1997
(51) Int. Cl.: B05D 7/24, B05D 3/14

(54) **PROCESS FOR MAKING A PARYLENE COATING**
VERFAHREN ZUR HERSTELLUNG EINER PARYLENBESCHICHTUNG
PROCEDE DE FABRICATION DE REVETEMENT A BASE DE PARYLENE

(30) Priority: 25.10.1996 US 738319; 12.09.1997 US 928931
(43) Date of publication of application: 11.08.1999
(73) Proprietor: SPECIALTY COATING SYSTEMS, INC., Indianapolis, Indiana 46241 (US)
(72) Inventor: WARY, John, Noblesville, IN 46060 (US); OLSON, Roger, A., Amery, WI 54001 (US); BEACH, William, F., Bridgewater, NJ 08807 (US)
(74) Representative: Allard, Susan Joyce
(86) International application number: US9719294
(87) International publication number: WO9818570

(56) References cited:
- EP-A- 0 262 676
- FR-A- 2 079 414
- FR-A- 2 259 687
- US-A- 4 500 562
- US-A- 5 139 813
- US-A- 5 154 978
- US-A- 5 538 758
- KRASOVSKY A M ET AL: "DEPOSITION OF POLY-P-XYLYLENE FILMS BY PLASMA DECOMPOSITION OF CYCLODI-P-XYLYLENE" JOURNAL OF APPLIED POLYMER SCIENCE, vol. 57, no. 1, 5 July 1995, pages 117-119, XP000541093
- DATABASE WPI Section Ch, Week 9442 Derwent Publications Ltd., London, GB; Class A26, AN 94-339549 XP002057052 & SU 1 819 687 A (AS BELO METAL POLYMER SYSTEMS MECH INST) , 7 June 1993
- PATENT ABSTRACTS OF JAPAN vol. 095, no. 004, 31 May 1995 & JP 07 014675 A (TOPPAN PRINTING CO LTD), 17 January 1995,
- PATENT ABSTRACTS OF JAPAN vol. 097, no. 007, 31 July 1997 & JP 09 071672 A (FUJI ELECTRIC CO LTD), 18 March 1997,
- DATABASE WPI Section Ch, Week 9410 Derwent Publications Ltd., London, GB; Class A26, AN 94-080770 XP002057051 & RU 2 002 519 C (AS BELO METAL POLYMER SYSTEMS MECH INST) , 15 November 1993
- CHOW S W ET AL: "POLY(ALPHA,ALPHA,ALPHA',ALPHA'-TETRAFLUOR O-P-XYLYLENE)" JOURNAL OF APPLIED POLYMER SCIENCE, vol. 13, no. 9, 1969, pages 2325-2332, XP000612619

## Description

### BACKGROUND OF THE INVENTION

### 1. Field Of The Invention

The present invention relates to a method of forming a parylene polymer layer according to the precharacterising part of claim 1 and to a multi-level structure according to the precharacterising part of claim 20.

### 2. Discussion Of The Related Art

Semiconductors are widely used in integrated circuits for electronic products systems such as computers and televisions. These integrated circuits typically combine many transistors on a single crystal silicon chip to perform complex functions and store data. Semiconductor and electronics manufacturers. as well as end users, desire integrated circuits which can accomplish more in less time in a smaller package while consuming less power. However, some of these desires may be in opposition to each other. For example, simply shrinking the feature sizes on a given circuit from 0.5 microns to 0.25 microns can increase power consumption by 30%. Likewise, doubling operational speed generally doubles power consumption. Miniaturization also generally results in increased capacitive coupling, or cross talk, between conductors which carry signals across the chip. This can limit achievable speed and degrade the noise margin used to insure proper device operation.

One way to diminish power consumption and cross talk effects is to decrease the dielectric constant of electrically insulating layers that separate layers of electrically conductive materials within the integrated circuit. In addition, since operational conditions may include high temperatures, it can be advantageous to use materials with relatively high thermal stability to form the insulating layers.

Silicon dioxide is one of the most common materials used in insulating layers for integrated circuits. However, silicon dioxide is non-ideal due to its comparatively high dielectric constant of about 3.9.

Layers formed from parylene polymers have been proposed for use as insulating layers in integrated circuits because these materials have relatively low dielectric constants and comparatively high melting temperatures. Parylene polymers are poly-p-xylylenes which may be prepared starting with a dimer having the structure: wherein X is typically a hydrogen or a halogen. The most common forms of parylene dimers include the following:

Polymer films formed from these parylene dimers may have comparatively low dielectric constants and relatively high melting temperatures. However, these parylene polymer films have relatively high dielectric constants and inferior thermal stabilities, rendering them less attractive for use in integrated circuits.

Typically, a vapor deposition method is used to form parylene polymer layers from parylene dimers. One such vapor deposition method is disclosed in *Journal of Applied Polymer Science* **13**, 2325 (1969). According to this method, commonly referred to as the Gorham process, the parylene dimer is cracked at an elevated temperature to produce parylene monomer having the structure:

The paryiene monomer is condensed onto a substrate at a temperature of from about room temperature to about -35 °C. Under these conditions, the parylene monomer simultaneously polymerizes on the substrate to form a layer of the parylene polymer adhered to the substrate.

This method is considered to be the closest prior art and is acknowledged in the preamble of the claims.

A vapor deposition process for forming poly-p-xylylene films from other than parylene dimer materials is disclosed in U.S. Patent No. 5,268,202 (You). The method disclosed by this reference includes forming the monomer vapor inside the vacuum chamber in which deposition occurs, precluding the purification opportunities afforded by the parylene dimer process prior to deposition on the substrate. Therefore. the resulting poly-p-xylylene layers have relatively high impurity levels. For example. *Journal of Vacuum Science and Technology* A11(6). 3057 (1993) discloses that poly-p-xylylene films formed by the method of You have zinc impurity levels of about 3%. Such a comparatively high level of zinc impurity results in problems with the poly-p-xylylene film relating to, for example, increased dielectric constant, decreased surface resistivity, ion movement within the layer, film surface charging effects and/or electron storm formation when the poly-p-xylylene film is used within a multi-level structure. As a result, these poly-p-xylylene films cannot be used in integrated circuits.

Combining the use of a plasma with the deposition of a gaseous species has been used in many systems. For example, DUMIC Conference, February 11, 1997, ISMIC-222D/97/0098-105 (hereinafter "DUMIC") discloses the use of a pulsed plasma to manipulate the control of fluorocarbon thin films on silicon. This reference focuses on controlling the relative amounts of CE₃, CF₂ and CE, rater than any effects on the deposition rate, deposition efficiency or adhesion of the resulting surface. Furthermore, DUMIC does not disclose the use of a pulsed plasma in conjunction with the formation of a parylene polymer film. As known to those skilled in the art, variation in the parameters used in connection with a pulsed plasma (e.g., peak power amplitude, peak power frequency and duty cycle) is dependent upon the surface created during deposition.

The use of polymeric material such as parylene is known in the art. For example, European Patent Application 0262 676 describes an electron emission device in the form of a multilayer structure have an organic insulation layer in the form of a plasma polymerized film formed by a CVD method from polyparaxylene and hydrocarbon. Similarly, Krasovsky, A.M. et al. in "Deposition of Poly-P-Xylylene Films by Plasma Decomposition of Cyclodi-P-Xylylene". Journal of Applied Polymer Science, Vol. 57, July 5, 1995, No. 1, pp. 117-119 describes a deposition process of poly-p-xylylene films using a glow-discharge plasma rather than via the Gorham method. U.S. Patent No. 5,154,978 to Nakayama et al. describes a corrosion resistant rare-earth-iron magnet having a paraxlylene polymer film or a chloroparaxylylene polymer film formed on its surface using a plasma polymerisation technique. U.S. Patent No. 4,500,562 to Jahn et al. relates to the formation of poly-p-xylylene films using a modified form of the Gorham process. In this technique, a pyrolyzed diradical p-xylylene monomer is exposed to a low pressure plasma prior to deposition for the process of forming a poly-p-xylylene film. Similarly, SU 1819687 relates to the formation of poly-p-xylylene films in which a CO-laser is used in connection with an auxiliary plasma chamber in the deposition system. Finally, Patent Abstracts of Japan Publication No. 07014675 describes an organic thin film EL element that is stabilized against degradation due to oxygen and moisture by providing a sealed layer having a metal oxide, a metal fluoride or a blended material of these metals that is mixed with a polyparaxylylene polymer on a negative electrode. The polyparaxylylene film is described as a "plasma polymeric film".

It remains a challenge in the art to provide an electrically insulating layer for use in integrated circuits of electronic devices that has a relatively low dielectric constant and comparatively high melting temperature. It is a further challenge in the art to provide such an insulating layer which is formed from a parylene polymer.

Additional art relative to the invention or descriptive of the background invention is as follows:

European Patent Application 0,262,676 relates to an electronic emission device having a first metal layer, an insulating layer formed on the first metal layer, a second metal layer formed on the insulating layer and a means for applying voltage across the first and second metal layers. The insulating layer is an organic insulating layer and may be from the parylene polymer.

Krasovsky et al., "Deposition of Poly-p-xylylene Films by Plasma Decomposition of Cyclodi-p-xylylene," *Journalof Applied Polymer Science,* Vol. 57, July 1995, Number 1, pp 117-119 describes the deposition of poly-p-xylylene films on surfaces using the Gorham method.

U.S. Patent No. 5,154,978 to Nakayama et al. relates to highly corrosion-resistant rare earth iron magnets. During the process used to form the magnets, a plasma treatment is employed.

U.S. Patent No. 4,500,562 to Jahn et al. relates to di-p-xylylene polymers and methods for making such polymers. These polymers are desposited onto a surface using a method such as the Gorham method. In describing the deposition of a di-p-xylylene polymer onto a surface, this reference can be said to form the basis of the preambles of the independent claims herein.

Soviet publication 1,819,687 relates to a method for depositing a poly-p-xylylene onto a surface. The xylylene is plasma-treated prior to the deposition.

Japanese abstract publication 07-014675 relates to an organic thin film EL element. The reference describes the deposition of a poly-p-xylylene on a surface.

French publication 2,079,414 describes the deposition of a "p-xylene" onto a surface.

French publication 2,259,687 describes a process in which a coating on a surface is hardened using a luminescent discharge.

U.S. Patent No. 5,139,813 to Yira et al. refers to a method for reducing flourescence in parylene films by an active plasma. In this method, a parylene coating on an article is exposed to a plasma for a period of time sufficient to produce flourescence in the surface layer of the parylene.

Japanese abstract 09-071672 relates to a method for modifying polyparaxylylene thin films to enhance their heat resistance. The method includes fluorinating the thin film by exposing the film to a plasma gas consisting mainly of CF₄.

U.S. Patent No. 5,538,758, naming the same inventors as those of the present invention, relates to a method and apparatus for the deposition of parylene AF4 onto semiconductor wafers. In describing the deposition of a flourinated parylene onto a surface, this reference serves, at least in part, as the basis for the preamble of the independent claims herein.

### Summary of the Invention

It is the object of the present invention to provide adhesion - promoting, substantially pure parylene polymer layers on substrate surfaces, the improved parylene polymer layers having relatively low levels of impurities such as, for example, zinc. In a first aspect, the above object is attained according to the invention by a method of forming a parylene polymer layer, which method comprises the step of depositing a monomer of parylene onto the surface of a substrate (12) to form a parylene polymer film layer (14), the parylene polymer having the structure parylene wherein
m has a value of 0, 1, 2, 3 or 4,
z is greater than 1,
G is a halogen atom, an alkyl group, a cyclohydrocarbon, an alkylene group or an akylyne group having the general formula CnHyXw wherein X is a halogen atom, n is greater than zero and the sum of y and w is at the most equal to 2n + 1,
characterized in that the parylene polymer film layer formed by treatment of the parylene monomer deposited on the surface with a pulsed plasma treatment.

In a second aspect, the above object is attained by a multi-level structure as defined in claim 20.

Particular embodiments of the invention are the subject of the respective dependent claims.

The structure comprises a first layer, a parylene polymer layer and a layer of adhesion promotion material. The parylene polymer layer is disposed along the first layer, and the layer of adhesion promotion material is disposed along the layer of adhesion promotion material. The parylene polymer layer is formed form a material that has a structure: wherein m is an integer having a value of 0, 1, 2, 3 or 4, z is greater than 1, G is a halogen, an alkyl group, a cyclo hydrocarbon, an alkylene group or an alkylyne group having the general formula CₙH_{y}X_{w}, wherein X is a halogen, n is an integer greater than zero and a sum of y and w is at most equal to a sum of 2n and 1, and wherein the parylene polymer layer has a zinc impurity level of at most about 66 parts per billion.

In yet another illustrative embodiment, the present invention provides a method making a multi-level structure. The method comprises depositing a monomer on the surface of a substrate to form a layer, and treating the layer with a pulsed plasma treatment to form a parylene polymer film on the surface of the first layer. The parylene polymer has a structure: wherein m is an integer having a value of 0, 1, 2, 3 or 4, z is greater than 1, G is a halogen, an alkyl group, a cyclo hydrocarbon, an alkylene group or an alkylyne group having the general formula CₙH_{y}X_{w}, wherein X is a halogen, n is an integer greater than zero and a sum of y and w is at most equal to a sum of 2n and 1, and wherein the parylene polymer layer has a zinc impurity level of at most about 66 parts per billion.

In a further illustrative embodiment, the present invention provides a multi-level structure. The structure comprises a first layer and a parylene polymer layer disposed along the surface of the first layer. The parylene polymer layer is formed from a material having a structure: wherein m is an integer having a value of 0, 1, 2, 3 or 4, z is greater than 1, G is a halogen, an alkyl group, a cyclo hydrocarbon, an alkylene group or an alkylyne group having the general formula CₙH_{y}X_{w}, wherein X is a halogen, n is an integer greater than zero, and a sum of y and w is at most equal to a sum of 2n and 1, and wherein the parylene polymer layer has a zinc impurity level of at most about 66 parts per billion. The parylene polymer layer is formed by a process including the steps of: depositing monomers of parylene onto a surface of a substrate to form a layer; and treating the layer with a pulsed plasma treatment.

The present invention provides a multi-level structure, comprising:
a first layer (12) having a surface; and
a parylene polymer layer (14) having first and second surfaces, the first surface of the parylene polymer layer being opposite to the second surface of the parylene polymer layer, the first surface of the parylene polymer layer being deposited along the surface of the first layer, the parylene polymer layer being formed from a material having a structure: wherein
   m has a value of 0, 1, 2, 3 or 4,
   z is greater than 1,
   G is a halogen atom, an alkyl group, a cyclohydrocarbon, an alkylene group or an akylyne group having the general formula CnHyXw wherein X is a halogen atom, n is greater than zero and the sum of y and w is at the most equal to 2n + 1,
characterized in that the parylene polymer layer has a zinc impurity level of at the most about 66 parts per billion and in that a layer of adhesion promoting material (16, 18) having a first surface and a second surface is provided, the first surface of the layer of adhesion promoting material being disposed along the second surface of the parylene polymer layer.

### BRIEF DESCRIPTION OF THE DRAWINGS

The advantages and features of the present invention will be more clearly understood in view of the following detailed description when taken in conjunction with the drawings, in which:
Fig. 1 is a cross-sectional view of one embodiment of a multi-level structure according to the present invention;
Fig. 2 is a cross-sectional view of another embodiment of a multi-level structure according to the present invention;
Fig. 3 is a block diagram of one embodiment of a vacuum deposition system which may be used to form parylene polymer layers according to the present invention;
Fig. 4 is a cross-sectional view of a portion of one embodiment of an integrated circuit including a multi-level structure according to the present invention; and
Fig. 5 is a block diagram of one embodiment of a vacuum chamber which may be used to form parylene polymer layers according to the present invention.

### DETAILED DESCRIPTION

Fig. 1 depicts a multi-level structure 10 according to the present invention. Structure 10 includes substrate layer 12 and parylene polymer layer 14. By "parylene polymer" it is herein meant to refer to a poly-p-xylylene. Typically, a parylene polymer is formed from a parylene dimer.

Substrate layer 12 may be formed from any materials onto which parylene polymer layer 14 is capable of being deposited. These materials may include electrically conductive and electrically non-conductive materials. The particular material from which layer 12 is formed depends upon the application, and such materials are known to those skilled in the an. For example, substrate layer 12 may be formed from organic materials or inorganic materials including, but not limited to, aluminum, iron, steel, molybdenum, aluminum oxide, titanium oxide, lead oxide, copper oxide, iron oxide, beryllium oxide, manganese oxide, tungsten oxide, tantalum oxide, vanadium oxide, silicones, natural rubbers, plastics, plastic composites, ceilulosic materials, epoxy-containing compounds, thermosetting compounds, thermoplastic compounds, oxides of silicon (e.g., fly ash, hydrated silica, silica, quartz, aerogels, Nerogels and fumed silica) and the like. Furthermore, layer 12 may comprise gallium arsenide or other binary semiconductors.

Substrate layer 12 may also be formed from a vacuum compatible liquid. By "vacuum compatible" it is herein meant to refer to a material that has a vapor pressure at the operating temperature of the vacuum chamber used such that the minimum pressure to which the vacuum chamber can be pumped is independent of the presence of the vacuum compatible material. One example of a vacuum compatible liquid is gamma-methacryloxypropyltrimethoxysilane.

In certain embodiments, substrate layer 12 may be a printed circuit board, a silicon backboard, a fiberglass backboard, a silicon wafer, paper, a key pad, a catheter, a pacemaker cover, a subcutaneous probe, a bird feather, a silicone 0-ring, parts of a mechanical apparatus, such as an automobile, or the like.

Parylene polymer layer 14 is formed from a material having the structure: m is an integer having a value of 0, 1, 2, 3 or 4, and z is greater than 1. G is a halogen, an alkyl group, a cyclo hydrocarbon an, alkylene group or an, alkylyne group having the general formula CₙH_{y}X_{w}, wherein X is a halogen, n is an integer greater than zero and z is 1. If G is an alkyl group (i.e., saturated) then y +w = 2n+1. If G is a cyclo hydrocarbon, an alkylene or alkylyne group (i.e., G has at least one degree of unsaturation) then y + w is less than 2n+1 by a factor of twice the degree of unsaturation.

Fig. 2 depicts another multi-level structure 20 according to the present invention. Structure 20 includes parylene polymer layer 14 disposed between a first layer of material 16 and a second layer of material 18. Although not limited to these materials, layers 16 and 18 may be formed from any of the materials listed above with reference to substrate layer 12. Furthermore, layer 16 and/or layer 18 may take on any of the above-noted shapes of substrate layer 12. Layer 16 and/or layer 18 may take on other shapes as well.

In certain embodiments, each of layers 16 and 18 may be formed from materials that are at least partially electrically conductive. In such embodiments, layers 16 and 18 may be formed from metals using standard photolithographic and etching techniques. For these embodiments, layers 16 and 18 may each correspond to a power plane, a ground plane or a metal interconnection trace layer. Other processes for forming layers 16 and 18 are known to those skilled in the art and are intended to be within the scope of the present invention.

In some embodiments, parylene polymer layer 14 may be relatively difficult to adhere to certain other materials. For these embodiments, it may be desirable to promote the adhesion of layer 14 to other surfaces. Accordingly, parylene polymer layer 14 may undergo certain surface treatments to increase its ability to adhere to other surfaces. Such treatments include, for example, continuous plasma treatment (i.e., substantially 100% duty cycle), corona treatment, charge treatment and/or other surface roughening treatments. These treatments are known to those skilled in the art and are intended to be within the scope of the present invention. For example, in a continuous plasma treatment, a radio frequency (RF) generator can be used in conjunction with a background pressure of one or more gases to produce a plasma.

During parylene monomer deposition, a pulsed plasma treatment has been found to increase the adhesion of the parylene monomer. By "pulsed plasma treatment" it is herein meant to refer to a plasma treatment in which the duty cycle (i.e., the percentage of time that the plasma is on during the treatment) is less than about 100%. Typically, the duty cycle of a pulsed plasma treatment is at most about 50%. Preferably, the duty cycle of a pulsed plasma treatment is from about 0.1% to about 50%, more preferably from about 0.1% to about 10% and most preferably about 0.2%.

Fig. 3 shows a block diagram of one embodiment of a vacuum system 80 having a pulsed plasma source appropriate for use in forming parylene polymer layers according to the present invention. System 80 includes a parylene monomer source 82, a deposition chamber 84, a substrate 86, and a platen 88 (see discussion below). In addition, system 80 includes a pulsed plasma source 90 connected to chamber 84 to allow a parylene polymer layer disposed on substrate 86 to undergo a pulsed plasma treatment. Pulsed plasma source 90 includes an RF generator 92 (model 300-1 RF generator, available from Technics Company, located in Alexandria, VA). A timing module 93 (model DMP10-.1-.4, available from Dynatronics, Inc., located in Amery, WI) interfaces pulsed plasma source 92 to a timing circuit 94 to control the duty cycle of the pulsed plasma treatment. Such timing circuits 94 are known to those skilled in the art. Furthermore, while particular examples of an RF generator and a timing module are disclosed herein, other such devices are known to those skilled in the art and are intended to be within the scope of the present invention.

During a pulsed plasma treatment, a background pressure of parylene monomer (e.g., from about 1.33 to about 0.20N/m² (about 10 to about 15 millitorr)) is present in chamber 82. As the parylene monomer is deposited on the surface of substrate 86, a pulsed plasma treatment occurs such. For example, if the duty cycle of the pulsed plasma is about 0.2%, the RF generator is on about 0.2% of the time that the parylene monomer is being deposited on the surface of substrate 86. Within the plasma, various ions, radicals and other species are formed from the parylene monomer gas. These species generally have high sticking coefficients and deposit on the surface of substrate 86 with high efficiency, resulting in a parylene polymer layer having enhanced properties as described herein.

The peak power of RF generator 92 during a pulsed plasma treatment can be varied depending upon the desired properties of the resulting parylene polymer layer. Generally, this peak power depends upon the volume of the deposition chamber, with the peak power increasing as the volume of the deposition chamber increases. If the peak power of generator 92 is too low, the pulsed plasma treatment may have minimal effect on improving the properties of a parylene polymer layer. However, if the peak power of generator 92 is too high, the resulting parylene polymer layer may be brittle, nontransparent or otherwise have undesirable properties. Accordingly, the peak power of RF generator 92 during a pulsed plasma treatment relative to the volume of the deposition chamber is preferably from about 0.003Js⁻¹cm⁻³ (about 0.05 Watts/inch³) to about 6Js⁻¹cm⁻³ (about 100 Watts/inch³), more preferably from about 0.006Js⁻¹cm⁻³ (about 0.1 Watts/inch³) to about 1.2Js⁻¹cm⁻³ (about 20 Watts/inch³) and most preferably from about 0.006Js⁻¹cm⁻³ (about 0.1 Watts/inch³) to about 0.6Js⁻¹cm⁻³ (about 10 Watts/inch³).

The increased adhesion associated with using a pulsed plasma treatment during parylene monomer deposition results in an increased thickness of the resulting parylene polymer film and an increased rate of deposition of the parylene monomer.

While holding other variables constant, relative to a parylene polymer film formed without a pulsed plasma treatment, a parylene polymer layer formed using a pulsed plasma treatment is preferably at least about 1.5 times as thick, more preferably at least about 2 times as thick and most preferably at least about 3 times as thick.

While holding other variables constant, relative to a parylene polymer film formed without a pulsed plasma treatment, the deposition rate of parylene monomer using a pulsed plasma treatment is preferably at least about 1.5 fast, more preferably at least 2 times as fast and most preferably at least 3 times as fast.

Surprisingly, in addition to providing enhanced adhesion, it has been found that treating the surface of a parylene polymer layer using a pulsed plasma results in other advantages. One such advantage relates to improved control over the surface onto which the parylene polymer layer is formed. Usually, when forming a parylene polymer layer on a substrate for use in the electronics industry, it is desirable to leave an area of about 1 mm thickness around the edge of the substrate that is substantially free of parylene polymer. This concept is commonly referred to within the art as edge exclusion. In addition, it is advantageous to minimize the amount of parylene polymer that forms on the underside of a substrate (i.e. on the side that is not directly facing the parylene monomer gas). Problems with accomplishing these goals can occur as a result of the deposition process in which the substrate is typically clamped to a platen at only a select few locations (e.g., 6 locations), such as described in commonly assigned U.S. Patent No. 5,546,473, which is herein incorporated by reference. Surprisingly, it has been found that enhanced edge exclusion and reduced parylene polymer formation on the underside of the substrate are achieved when a parylene polymer layer undergoes pulsed plasma treatment relative to parylene polymer layers that undergo no plasma treatment or continuous plasma treatment.

An additional advantage to using a pulsed plasma treatment when forming a parylene polymer layer relates to the dielectric constant of the resulting parylene polymer layer. In many embodiments, such as when the parylene polymer layer is used as an insulating layer, such as in the electronics industry, it is advantageous for the parylene polymer layer to have a minimal dielectric constant. Furthermore, it is often desirable that the in-plane dielectric constant (i.e. the dielectric constant parallel to a plane of the substrate) and out-of-plane dielectric constant (i.e. the dielectric constant in a plane perpendicular to the substrate) of the parylene polymer layer be approximately equal. Unexpectedly, it has been found that pulsed plasma treatment of a parylene polymer layer results in a parylene polymer layer with reduced dielectric constants relative to the dielectric constants of parylene polymer layers formed with no plasma treatment or with a continuous plasma treatment, and, surprisingly, the values of the in-plane dielectric constants and out-of-plane dielectric constants of parylene polymer layers formed using pulsed plasma treatment are closer to the same than the values of the in-plane and out-of-plane dielectric constants for parylene polymer layers formed with no plasma treatment or with a continuous plasma treatment. Hence, relative to a parylene polymer layer formed without using a pulsed plasma treatment, a parylene polymer layer formed using a pulsed plasma treatment can have a reduced dielectric constant and/or a dielectric constant that is more isotropic. Pulsed plasma treatment or continuous plasma treatment of a parylene polymer layer can be performed during or after parylene monomer deposition. In addition, during a plasma treatment, a background pressure of a gas other than parylene monomer (i.e. a background gas) can be present. Preferably, the pressure of the background gas in the deposition chamber is from about 16.6N/m² to about 49.9N/m² (about 125 millitorr to about 375 millitorr), more preferably from about 26.6N/m² to about 39.9N/m² (about 200 millitorr to about 300 millitorr) and most preferably from about 31.9N/m² to about 34.6 N/m² (about 240 millitorr to about 260 millitorr). In some embodiments, a background gas is comprised of one or more noble gases. Examples of noble gases include helium, neon, argon and xenon. In other embodiments, a background gas can include one or more hydrocarbons. Such hydrocarbon background gases may be saturated hydrocarbons, unsaturated hydrocarbons, aromatic hydrocarbons, straight-chained hydrocarbons, branched hydrocarbons, cyclic hydrocarbons and the like. An exemplary list of hydrocarbons appropriate for use as background gases includes, but is not limited to, methane, ethane, ethylene and acetylene. In certain embodiments, a background gas can comprise one or more noble gases and one or more hydrocarbon gases. It has been found that the use of one or more hydrocarbon gases results in parylene polymer layers having improved properties (see discussion below).

It is to be understood that the aforementioned treatments of parylene polymer layers may be performed on an entire parylene polymer layer or a portion of a parylene polymer layer. In addition, while certain treatments of parylene polymer layers have been disclosed herein, it is to be understood that other treatments of parylene polymer layers to enhance adhesion, or other properties, of these layers will be apparent to those skilled in the art and are intended to be within the scope of the present invention.

Parylene polymers are usually highly crystalline and linear materials, which can limit the strength or other physical properties of these layers. To improve the strength of a parylene polymer layer, additional chemical species (e.g., monomers) other than parylene monomer, may be added to the layer during synthesis of the layer. When incorporated into the parylene polymer layer, these additional components should allow cross-linking to occur, increasing the strength and/or adhesion of the resulting layer. An illustrative and nonlimiting list of such chemical species includes species having a molecular formula CₓH_{y} where each of x and y is an integer of at least one.

Incorporation of these chemical species into a parylene polymer layer can be accomplished by, for example, establishing a background pressure of these other components within the deposition chamber during parylene monomer deposition. In certain embodiments, a pulsed plasma treatment or continuous plasma treatment can be used when a background pressure of one or more of these chemical species is present in the deposition chamber, but such pulsed plasma treatment or continuous plasma treatment is not required.

In embodiments of the present invention in which a chemical species other than parylene monomer is incorporated into a parylene polymer, the parylene polymer preferably should have an amount of the chemical species incorporated therein to improve the properties of the parylene polymer layer such that at least one of the advantages of the present invention as described herein is attained.

In some embodiments, enhanced adhesion may be achieved by providing a layer of adhesion promoting material between layer 16 and layer 14 and/or between layer 18 and layer 14. Alternatively, layer 16 and/or layer 18 may be formed from an adhesion promotion material. Adhesion promotion materials appropriate for use in the present invention include, but arc not limited to, organosilane compounds, metals, metal oxides and semiconductor oxides. Examples of such organosilane compounds include A-150 (available from Union Carbide Technologies), A-174 (available from Union Carbide Technologies) and VM 651 (available from DuPont Chemicals). Other such adhesion promotion materials are known to those skilled in the art and are intended to be within the scope of the present invention. It is to be appreciated that, for these embodiments, layer 14 may or may not undergo any of the above-noted surface treatments.

For some applications, it may be advantageous to prevent the diffusion of materials through parylene polymer layer 14. For these applications, layer 16 and/or layer 18 may be formed from materials that reduce or eliminate the diffusion of materials through parylene polymer layer 14. Materials appropriate for use in these applications are disclosed in, for example, U.S. Patent No. 5,470,802. Other such materials are known to those skilled in the art and are intended to be within the scope of the present invention.

For certain uses, such as, for example, electronic circuits, it may be desirable to form relatively flat layers, but, since parylene polymer layer 14 is comparatively conformal, layer 14 may not have the desired degree of flatness. Hence, it may be advantageous to grind or otherwise treat layer 14 to make it more flat, often referred as planarizing within the art. However, in certain embodiments, layer 14 may be difficult to planarize. For these embodiments, layer 16 and/or layer 18 may be formed from a material that is more readily planarized. Typically, such a material is a dielectric material, but, in some instances, it may be an electrical conductor.

Fig. 4 shows a portion 30 of a multi-level electronic circuit according to the present invention. Portion 30 includes silicon wafer substrate 22, electrically insulating layer 24, electrically conductive layer 26, electrically conductive layer 28 and parylene polymer layer 14 disposed between layers 26 and 28.

Silicon wafer substrate 22 may be formed from any of the standard substrate materials used in the electronics industry, such as, for example, a silicon backboard or a fiberglass backboard. Other appropriate structures for wafer substrate 22 are known to those skilled in the art and are intended to be within the scope of the present invention.

Electrically insulating layer 24 typically functions to protect wafer substrate 22 from electrically conductive layers 26 and 28. Layer 24 is usually formed from silicon dioxide, although other appropriate materials may be used. Electrically insulating layer 24 may be formed according to any of the standard techniques known to those skilled in the art.

Electrically conductive layers 26 and 28 may be formed from metals or other materials appropriate for use in electronic circuits. Layers 26 and 28 may comprise metal conductor lines which are formed according to standard photolithographic and etching techniques. For such embodiments, layers 26 and 28 may each, correspond to a power plane, a ground plane or an interconnection trace layer.

Electrically conductive layers 26 and 28 may be interconnected through parylene polymer layer 14 by use of vias, or through holes (not shown), which are formed in parylene polymer layer 14 by conventional processes known to those skilled in the art.

According to the present invention, parylene polymer layer 14 is formed using a vapor deposition process. Preferably, the vapor deposition process allows the monomer to be formed outside the deposition portion of the vacuum chamber such that the monomers can undergo a purification process prior to being deposited onto the substrate. In a particularly preferred embodiment, parylene polymer layer 14 is formed using a vacuum chamber 40 as depicted in Fig. 5. Vacuum chamber 40 includes vaporization zone 42, a pyrolysis zone 44, a post-pyrolysis zone 46 and a deposition zone 48. Examples of such vacuum chamber arc disclosed in, for example, commonly assigned U.S. Patent No. 5,546,473, which is herein incorporated by reference.

A dimer material having the structure: is placed within vaporization zone 42 at about room temperature and subsequently heated to a temperature of from about 70°C to about 150°C to vaporize the dimer.

The vaporized dimer passes into pyrolysis zone 44 which is maintained at a temperature of from about 600°C to about 720°C to pyrolize the dimer (i.e. cleave certain chemical bonds) and form a monomer having the following structure:

The monomer passes through post-pyrolysis zone 46 which is maintained at a temperature of at most about room temperature. At this temperature, residual vaporized dimer can adhere to the walls of post-pyrolysis zone 46 while the monomer generally passes through post-pyrolysis zone 46 without adhering to the walls of zone 46. Thus, post-pyrolysis zone 46 reduces the amount of vaporized dimer that ultimately enter deposition chamber 48. In certain embodiments, this feature can be advantageous because the vaporized dimer can constitute an impurity in parylene polymer layer 14, which may have an undesirable local effect on the dielectric constant or other properties of layer 14.

After passing through post-pyrolysis zone 46, the monomer enters deposition chamber 48 which includes substrate 50. Substrate 50 is placed on a platen 52 that includes a standard temperature controlling device 54 that controls the temperature by the platen by heating and/or cooling platen 54. By use of device 54, the temperature of substrate 50 and platen 52 is typically held at a temperature of from about room temperature to about -25°C during deposition of the monomer onto substrate 50.

It has been found that reducing the temperature of substrate 50 and platen 52 during monomer deposition can provide several advantages, including more control of the overall process of making parylene polymer layer 14 by allowing for increased manipulation of the monomer. For example, cooling substrate 50 and platen 52 allows for the walls of deposition chamber 48 to be heated during monomer deposition. In addition, reducing the temperature of substrate 50 and platen 52 during monomer deposition results in a more efficient deposition process and a more efficient use of the parylene dimer starting material.

Subsequent to monomer deposition, device 54 may be used to increase the temperature of substrate 50 and platen 52 to a temperature of from about 100°C to about 400°C to anneal the parylene polymer layer. However, it is to be noted that polymerization of the parylene monomer occurs spontaneously at the temperatures of substrate 50 noted above.

Prior to placing the dimer within vaporization zone 46, the dimer is first purified. Since the dimer of the present invention has a high degree of symmetry, it is readily purified by crystallization. Typically, these solvents are relatively unsymmetric in order to have a high temperature coefficient of solubility. However, if the solvent is too symmetric, separation of the solvent from the dimer may be difficult. Without wishing to be bound by any theories, it is believed that this increased difficulty in solvent/dimer separation results from the accidental accommodation of the solvent within the dimer lattice. Solvents appropriate for use in dimer crystallization according to the present invention include, but are not limited to, chloroform, tetrahydrofuran, methylene chloride, and linear hydrocarbons such as n-hexane and n-heptane. In a preferred embodiment, the solvent is n-hexane. After dissolving the dimer in the solvent, this solution is typically passed through a chromatographic bed including a polar material such as, for example, alumina. The polar nature of the chromatographic bed removes many of the polar or ionic impurities present within the solution. Furthermore, the chromatographic bed can remove fine impurities within the solution by filtration.

Using this process has been found to produce parylene polymer layers which have reduced levels of impurities. For example, parylene polymer layers in accordance with the present invention may have zinc impurity levels of 66 parts per billion or less. This feature of the present invention is desirable because impurities within parylene polymers can result in several different negative effects, including, but not limited to, an increase in the dielectric constant of the parylene polymer layer, a decrease in the surface resistivity of the parylene polymer layer and/or electron storm formation within the multi-level structure.

While particular apparatuses and methods of making parylene polymer layer 14 have been described herein, one skilled in the art would understand that at least certain aspects of these apparatuses and methods may be varied or modified, and such variations and modifications are intended to be within the scope of the present invention. For example, in addition to cleaving the parylene dimer bond by use of elevated temperature as discussed above, the parylene dimer may be cleaved by use of a plasma. Such methods are disclosed in, for example, Russian Patent Nos. RU 2,000,850 and RU 2,002,519.

When used in integrated circuits or for other electronics applications, parylene polymer layer 14 should have a minimal dielectric constant to enhance circuit operating speed and decrease power consumption. Accordingly, these parylene polymer layers preferably have a dielectric constant of at most about 2.6, more preferably at most about 2.4 and most preferably at most about 2.2.

Having a low dissipation factor decreases the signal loss in an integrated circuit. Therefore, parylene polymer layers in accordance with the present invention preferably have a dissipation factor of less than about 0.001.

According to the present invention, parylene polymer layers with a thickness of about one micrometer preferably have a breakdown voltage of at least about 750 volts.

Parylene polymer layer 14 preferably has a Young's modulus of about 5x10⁹N/m², (about 5 gigapascals). The elongation to break of parylene polymer layers according to the present invention is preferably at least about 20%.

Parylene polymer layer 14 preferably has an ultimate tensile strength of at least about 1.22x10⁸N/m², (about 122 megapascals).

According to the present invention, parylene polymer layers have water absorption values of at most about 0.5% by weight, more preferably at most about 0.2% by weight and most preferably at most about 0.1% by weight.

Parylene polymer layers in accordance 'with the present invention preferably have a thermal stability such that these layers demonstrate less than 1% weight loss per 2 hours at a temperature of at least about 450°C.

Parylene polymer layer 14 preferably has a crystalline melting point of above about 500°C.

The surface resistivity of parylene polymer layers in accordance with the present invention is preferably about 1.3x10¹⁴ ohms.

The volume resistivity of parylene polymer layer 14 is preferably about 5.3x10¹⁶ ohms.

Parylene polymer layers in accordance with the present invention preferably have a density of about 1.58.

The thermal expansion at 25°C of parylene polymer layer 14 is preferably at most about 35 parts per million.

According to the present invention, parylene polymer layers have a coefficient of friction of about 0.2.

The following are illustrative examples of embodiments of the present invention. They are not to be construed as limiting.

### Example 1

The following process was performed in a jacketed Soxhlet extractor (available as catalog number LG-6950, from Lab Glass, located in Vineland, NJ or as catalog number CG-1328, available from Chem Glass, located in Vineland, NJ). An amount of the crude dimer used as the starting material in the synthesis of the parylene polymer layers of the present invention was placed within a glass extraction thimble with a fritted glass disk at its bottom. A short chromatographic bed of particulate alumina was placed at the bottom of the thimble. The thimble was purchased with a diameter of 41 mm and a height of 130 mm. The height of the thimble was increased to 180 mm to accommodate larger samples (i.e., up to about 70 grams) of the crude dimer.

A flask of boiling n-hexane was placed below the thimble, and gaseous n-hexane was condensed in a condenser mounted above the thimble. The condensed n-hexane dripped onto the crude dimer to form a leachant solution of the condensed n-hexane, purified dimer and impurities, including dirt, dust, and/or polymers or oligomers of the monomer formed by the dimer. The leachant solution passed through the chromatographic bed and fritted glass at the bottom of the thimble. The chromatographic bed removed many polar or ionic impurities present within the leachant solution due to the polar nature of alumina. In addition, the chromatographic bed removed fine impurities by filtration.

A siphoning mechanism was used to periodically empty the leachant solution from the Soxhlet extractor holding the thimble. This process returned the n-hexane from the leachant solution to the flask of boiling n-hexane. After a period of from about 10 to about 20 hours, the crude dimer ended up in the flask of boiling n-hexane.

The extraction was conducted at the boiling n-hexane to speed up the dimer dissolution process. To accomplish this, a conduit jacket surrounded the extraction volume, so the extraction volume was heated by vapors of n-hexane as these vapors traveled from the boiling flask to the condenser. While this hot filtration process is advantageous because impurities are removed while the solution is hot, it is to be noted that, in conventional crystallization equipment, such a hot filtration can be difficult and/or dangerous when flammable solvents are used. Furthermore, for practical reasons, such a filtration may be performed at temperatures below the solvent boiling temperature, resulting in increased solvent use and decreased dimer solubility. However, using a Soxhlet apparatus, the boiling solvent vapors are held within the apparatus by the jacket, allowing for increased efficiency in the purification process.

The resulting purified dimer of the present invention was tested by inductively coupled plasma-mass spectrometry of the vaporized dimer. During this process, the sample is ashed to remove carbon containing components, leaving nonvolatile oxides of the trace elements to be determined. This ash is taken up in an aqueous buffer solution. The aqueous buffer solution of the sample ash is fed to an energized plasma. The high temperature of the plasma atomizes the trace elements. The atomized plasma is fed to the source of a mass spectrometer for quantification of each specific impurity elements.

The results are shown in Table 1, which clearly demonstrates that the zinc impurity levels are about 66 parts per billion. This method does not involve a direct measurement of the impurity level of the parylene polymer layer formed from the monomers. However, by measuring the impurity level of the starting material (i.e., dimer) for parylene polymer film synthesis, this method does provide an upper limit on the possible impurity level of the parylene polymer films of the present invention.

**Table 1**

| Element | Impurity Level (Parts per Billion) |
|---|---|
| Al | 460 |
| Ba | 6.2 |
| Be | <10 |
| Bi | <10 |
| Cd | <12 |
| Ca | 660 |
| Cs | 880 |
| Cr | 10 |
| Co | <1 |
| Cu | <5 |
| Ga | <1 |
| In | <1 |
| Fe | 140 |
| Pb | 7.4 |
| Li | 37 |
| Mg | 83 |
| Mn | 2.3 |
| Mo | <5 |
| Ni | 7.8 |
| K | 99 |
| Rb | <1 |
| Ag | <10 |
| Na | 500 |
| Sr | <1 |
| Th | <10 |
| Sn | 310 |
| V | <1 |
| Zn | 66 |
| Zr | <10 |

To purify about 70 grams of crude dimer according to this process, about 3 liters of n-hexane may be used. In this embodiment of the process, a 1 liter flask having an initial volume of about 0.7 1 of n-hexane is utilized.

### Example 2

A parylene polymer layer was formed was formed without a pulsed plasma treatment as follows. The deposition apparatus was as described in U.S. Patent No. 5,546,473. 0.5 grams of parylene dimer were placed into a crucible within the vaporization zone. The parylene dimer had the molecular structure: The crucible was heated to 105°C for thirty minutes, and the dimer was vaporized. The vaporized dimer passed into the pyrolysis zone which was held at 640°C. The dimer was pyrolized to form parylene monomer in the pyrolysis zone, and the parylene monomer was passed through the postpyrolysis zone which was held at - 100°C. Parylene monomer deposited on the surface of a six inch silicon wafer which was attached to a platen held at -15°C. The resulting parylene polymer layer had a thickness of 1 micrometer, and the deposition rate was 700Å per minute.

### Example 3

A parylene polymer layer was formed using the method described in Example 2, but a pulsed plasma treatment was used during the parylene monomer deposition. The resulting parylene polymer layer had a thickness of 3 micrometers, and the deposition rate was 2100Å per minute.

Having thus described particular embodiments of the present invention, various alterations, modifications and improvements will readily occur to those skilled in the art. Such alterations, modifications and improvements are intended to be part of this disclosure, and are intended to be within the scope of the present invention. Accordingly, the foregoing description is by way of example only and is not intended as limited. The present invention is limited only as defined by the following claims.

## Claims

1. A method of forming a parylene polymer layer, which method comprises the step of depositing a monomer of parylene onto the surface of a substrate (12) to form a parylene polymer film layer (14), the parylene polymer having the structure wherein
m has a value of 0, 1, 2, 3 or 4,
z is greater than 1,
G is a halogen atom, an alkyl group, a cyclohydrocarbon, an alkylene group or an akylyne group having the general formula CnHyXw wherein X is a halogen atom, n is greater than zero and the sum of y and w is at the most equal to 2n + 1,
**characterized in that** the parylene polymer film layer formed by treatment of the parylene monomer deposited on the surface with a pulsed plasma treatment.

2. A method as claimed in claim 1, wherein the depositing step and the treating step are performed simultaneously.

3. A method as claimed in claim 1, wherein the treating step is performed after the deposition step.

4. A method as claimed in any one of the preceding claims further comprising the step of establishing a pressure of a background gas sufficient to allow deposition of the background gas onto the surface of the substrate.

5. A method as claimed in claim 4, wherein the establishing step is performed simultaneously with the deposition step.

6. A method as claimed in claim 4 or claim 5, wherein the pressure of the background gas is from about 16.6N/m² to about 49.9N/m² (about 125 millitorr to 375 millitorr).

7. A method as claimed in claim 4 or claim 5, wherein the background gas is a hydrocarbon.

8. A method as claimed in claim 7, wherein the the background gas is methane, ethane, ethylene, acetylene, or mixtures thereof.

9. A method as claimed in any one of the preceding claims wherein the treatment step includes using a duty cycle of from 0.1% to 50%.

10. A method as claimed in claim 9, wherein the treating step includes using a duty cycle of from about 0.2% to about 10%.

11. A method as claimed in any one of the preceding claims wherein the treatment step includes using a peak power of from 0.003Js⁻¹cm⁻³ to 6Js⁻¹cm⁻³ (0.05 watts/inch³ to 100 watts/inch³).

12. A method as claimed in claim 11, wherein the treatment step includes using a peak power of from 0.006Js⁻¹cm⁻³ to 1.2Js⁻¹cm⁻³ (0.1 watts/inch³ to 20 watts/inch³).

13. A method as claimed in claim 11, wherein the treatment step includes using a peak power of from 0.006Js⁻¹cm⁻³ to 0.6Js⁻¹cm⁻³ (0.1 watts/inch³ to 10 watts/inch³).

14. A method as claimed in any one of the preceding claims the parylene polymer layer has a zinc impurity level of at the most about 66 parts per billion.

15. A method as claimed in any one of the preceding claims which comprises the steps of vaporizing a parylene dimer and pyrolyzing the parylene dimer to form the monomer.

16. A method as claimed in claim 15, wherein the depositing step occurs in a deposition zone (48) of a vacuum chamber (40).

17. A method as claimed in claim 15, wherein the pyrolyzing step occurs outside the deposition zone (48) of the vacuum chamber (40).

18. A method as claimed in any one of claims 15 to 17 further comprising the step of feeding the monomer into the deposition zone (48) of the vacuum chamber (40).

19. A method as claimed in any one of claims 15 to 18, wherein the polymerizing step includes polymerizing the monomer to form a parylene polymer film having a zinc impurity level of about 66 parts per billion.

20. A multi-level structure, comprising:
a first layer (12) having a surface; and
a parylene polymer layer (14) having first and second surfaces, the first surface of the parylene polymer layer being opposite to the second surface of the parylene polymer layer, the first surface of the parylene polymer layer being deposited along the surface of the first layer, the parylene polymer layer being formed from a material having a structure: wherein
m has a value of 0, 1, 2, 3 or 4,
z is greater than 1,
G is a halogen atom, an alkyl group, a cyclohydrocarbon, an alkylene group or an akylyne group having the general formula CnHyXw wherein X is a halogen atom, n is greater than zero and the sum of y and w is at the most equal to 2n + 1,
**characterized that** the parylene polymer layer has a zinc impurity level of at the most about 66 parts per billion and in that a layer of adhesion promoting material (16, 18) having a first surface and a second surface is provided, the first surface of the layer of adhesion promoting material being disposed along the second surface of the parylene polymer layer.

21. A multi-level structure as claimed in claim 20, wherein the adhesion promoting material is selected from the group consisting of organosilane compounds, metals, metal oxides, silicon oxides and semiconductor oxides.

22. A multi-level structure as claimed in claim 20 or claim 21, further comprising a second layer of an adhesion promoting material arranged in a manner such that the parylene polymer layer is disposed between the first and second layers of the adhesion promoting material.

23. A multi-level structure as claimed in claim 22 wherein the first adhesion layer is an electrically conductive material.

24. A multi-level structure as claimed in claim 22 wherein the second adhesion layer is formed from an electrically conductive material.

25. A multi-level structure as claimed in any one of claims 20 to 24, wherein the parylene polymer layer has a dielectric constant of at most about 2.6.

26. A multi-level structure as claimed in any one of claims 20 to 25, wherein the parylene polymer further includes a metallic species.

## Patentansprüche

1. Verfahren zum Bilden einer Parylenpolymerschicht, wobei das Verfahren den Schritt des Ablagerns eines Parylenmonomers auf der Oberfläche eines Substrats (12), um eine Parylenpolymerfilmschicht (14) zu bilden, umfaßt, wobei das Parylenpolymer die Struktur hat. wobei m einen Wert von 0, 1, 2, 3 oder 4 hat, z größer 1 ist, G ein Halogenatom, eine Alkylgruppe, ein Cyclokohlenwasserstoff, eine Alkengruppe oder eine Alkingruppe mit der allgemeinen Formel CnHyXw ist, worin X ein Halogenatom ist, n größer Null ist, und die Summe aus y und w höchstens gleich 2n + 1 ist,
**dadurch gekennzeichnet, daß** die Parylenpolymefilmschicht durch Behandlung des auf die Oberfläche abgelagerten Parylenmonomers mit einer · Plasmaimpulsbehandlung gebildet wird.

2. Verfahren nach Anspruch 1, wobei der Ablagerungsschritt und der Behandlungsschritt gleichzeitig durchgeführt werden.

3. Verfahren nach Anspruch 1, wobei der Behandlungsschritt nach dem Ablagerungsschritt durchgeführt wird.

4. Verfahren nach einem der vorhergehenden Ansprüche, weiterhin umfassend den Schritt des Einrichtens eines Drucks eines Hintergrundgases, der ausreichend ist um eine Ablagerung des Hintergrundgases auf der Oberfläche des Substrats zu ermöglichen.

5. Verfahren nach Anspruch 4, wobei der Einrichtschritt gleichzeitig mit dem Ablagerungsschritt durchgeführt wird.

6. Verfahren nach Anspruch 4 oder Anspruch 5, wobei der Druck des Hintergrundgases von etwa 16,6 N/m² bis etwa 49,9 N/m² (etwa 125 Millitorr bis 375 Millitorr) beträgt.

7. Verfahren nach Anspruch 4 oder Anspruch 5, wobei das Hintergrundgas ein Kohlenwasserstoff ist.

8. Verfahren nach Anspruch 7, wobei das Hintergundgas Methan, Ethan, Ethylen, Acetylen oder Gemische davon ist.

9. Verfahren nach einem der vorhergehenden Ansprüche, wobei der Behandlungsschritt die Verwendung eines Arbeitszyklus von 0,1% bis 50% umfaßt.

10. Verfahren nach Anspruch 9, wobei der Behandlungsschritt die Verwendung eines Arbeitszyklus von etwa 0,2% bis etwa 10% umfaßt.

11. Verfahren nach einem der vorhergehenden Ansprüche, wobei der Behandlungsschritt die Verwendung einer Spitzenleistung von 0,003 Js⁻¹cm⁻³ bis 6 Js⁻¹cm⁻³ (0,05 Watt/Zoll³ bis 100 Watt/Zoll³) umfaßt.

12. Verfahren nach einem der vorhergehenden Ansprüche, wobei der Behandlungsschritt die Verwendung einer Spitzenleistung von 0,006 Js⁻¹cm⁻³ bis 1,2 Js⁻¹cm⁻³ (0,1 Watt/Zoll³ bis 20 Watt/Zoll³) umfaßt.

13. Verfahren nach einem der vorhergehenden Ansprüche, wobei der Behandlungsschritt die Verwendung einer Spitzenleistung von 0,006 Js⁻¹cm⁻³ bis 0,6 Js⁻¹cm⁻³ (0,1 Watt/Zoll³ bis 10 Watt/Zoll³) umfaßt.

14. Verfahren nach einem der vorhergehenden Ansprüche, wobei die Paryienpolymerschicht einen Zinkverunreinigungsgrad von höchstens 66 Teilen pro Milliarde hat.

15. Verfahren nach einem der vorhergehenden Ansprüche, umfassend die Schritte des Verdampfens eines Parylendimers und des Pyrolysierens des Parylendimers, wobei das Monomer gebildet wird.

16. Verfahren nach Anspruch 15, wobei der Ablagerungsschritt in einer Ablagerungszone (48) einer Vakuumkammer (40) stattfindet.

17. Verfahren nach Anspruch 15, wobei der Pyrolyseschritt außerhalb der Ablagerungszone (48) der Vakuumkammer (40) stattfindet.

18. Verfahren nach einem der Ansprüche 15 bis 17, weiterhin umfassend den Schritt des Einbringens des Monomers in die Ablagerungszone (48) der Vakuumkammer (40).

19. Verfahren nach einem der Ansprüche 15 bis 18, wobei der Polymerisationsschritt das Polymerisieren des Monomers umfaßt, wobei ein Parylenpolymerfilm mit einem Zinkverunreinigungsgrad von höchstens 66 Teilen pro Milliarde gebildet wird.

20. Mehrebenenstruktur, umfassend:
eine erste Schicht (12) mit einer Oberfläche, und
eine Parylenpolymerschicht (14) mit einer ersten und zweiten Oberfläche, wobei die erste Oberfläche der Parylenpolymerschicht der zweiten Oberfläche der Parylenpolymerschicht gegenüberliegt, die erste Oberfläche der Parylenpolymerschicht auf der Oberfläche der ersten Schicht abgelagert ist, die Parylenpofymerschicht aus einem Material mit einer Struktur: gebildet ist, wobei m einen Wert von 0, 1, 2, 3 oder 4 hat, z größer 1 ist, G ein Halogenatom, eine Alkylgruppe, ein Cyclokohlenwasserstoff, eine Alkengruppe oder eine Alkingruppe mit der allgemeinen Formel CnHyXw ist, worin X ein Halogenatom ist, n größer Null ist, und die Summe aus y und w höchstens gleich 2n + 1 ist,
**dadurch gekennzeichnet, daß** die Parylenpolymerschicht einen
Zinkverunreinigungsgrad von höchstens etwa 66 Teilen pro Milliarde hat, und daß eine Schicht aus Haftvermittlermaterial (16, 18) mit einer ersten Oberfläche und einer zweiten Oberfläche bereitgestellt ist, wobei die erste Oberfläche der Schicht aus Haftvermittlermaterial auf der zweiten Oberfläche der Parylenpolymerschicht angeordnet ist.

21. Mehrebenenstruktur nach Anspruch 20, wobei das Haftvermittlermaterial ausgewählt ist aus der Gruppe, bestehend aus Organosilanverbindungen, Metallen, Metalloxiden. Siliziumoxiden und Halbleiteroxiden.

22. Mehrebenenstruktur nach Anspruch 20 oder Anspruch 21, weiterhin umfassend eine zweite Schicht aus Haftvermittlermaterial, welche derart angeordnet ist, so daß die Parylenpolymerschicht zwischen der ersten und zweiten Schicht des Haftvermittlermaterials angeordnet ist.

23. Mehrebenenstruktur nach Anspruch 22, wobei die erste Haftschicht ein elektrisch leitfähiges Material ist.

24. Mehrebenenstruktur nach Anspruch 22, wobei die zweite Haftschicht aus einem elektrisch leitfähigen Material gebildet ist.

25. Mehrebenenstruktur nach einem der Ansprüche 20 bis 24, wobei die Parylenpolymerschicht eine Dielektrizitätskonstante von höchstens etwa 2,6

26. Mehrebenenstruktur nach einem der Ansprüche 20 bis 25, wobei das Parylenpolymer weiterhin eine metallische Spezies umfaßt.

## Revendications

1. Procédé pour former une couche de polymère parylène, procédé qui comprend l'étape consistant à déposer un monomère parylène sur la surface d'un substrat (12) pour former une couche constituée d'un film de polymère parylène (14), le polymère parylène ayant la structure dans laquelle
m a la valeur 0, 1, 2, 3 ou 4,
z est supérieur à 1,
G représente un atome d'halogène, un groupe alkyle, un groupe hydrocarboné cyclique, un groupe alkylène ou un groupe alkylyne de formule générale CnHyXw dans laquelle X représente un atome d'halogène, n est supérieur à zéro et la somme de y et w est au plus égale à 2n + 1,
**caractérisé en ce que** la couche consistant en un film de polymère parylène est formée en traitant le monomère parylène déposé sur la surface par traitement par plasma pulsé.

2. Procédé suivant la revendication 1, dans lequel l'étape de dépôt et l'étape de traitement sont mises en oeuvre simultanément.

3. Procédé suivant la revendication 1, dans lequel l'étape de traitement est mise en oeuvre après l'étape de dépôt.

4. Procédé suivant l'une quelconque des revendications précédentes, comprenant en outre l'étape consistant à établir une pression d'un gaz de fond suffisante pour permettre le dépôt du gaz de fond sur la surface du substrat.

5. Procédé suivant la revendication 4, dans lequel l'étape d'établissement est mise en oeuvre simultanément avec l'étape de dépôt.

6. Procédé suivant la revendication 4 ou la revendication 5, dans lequel la pression du gaz de fond est comprise dans l'intervalle d'environ 16,6 N/m² à environ 49,9 N/m² (environ 125 millitorrs à 375 millitorrs).

7. Procédé suivant la revendication 4 ou la revendication 5, dans lequel le gaz de fond est un hydrocarbure.

8. Procédé suivant la revendication 7, dans lequel le gaz de fond est le méthane, l'éthane, l'éthylène, l'acétylène ou leurs mélanges.

9. Procédé suivant l'une quelconque des revendications précédentes, dans lequel l'étape de traitement comprend l'utilisation d'un cycle de fonctionnement de 0,1 % à 50 %.

10. Procédé suivant la revendication 9, dans lequel l'étape de traitement comprend l'utilisation d'un cycle de fonctionnement d'environ 0,2 % à environ 10 %.

11. Procédé suivant l'une quelconque des revendications précédentes, dans lequel l'étape de traitement comprend l'utilisation d'une puissance maximale de 0,003 Js⁻¹cm⁻³ à 6 Js⁻¹cm⁻³ (0,05 watt/inch³ à 100 watts/inch³).

12. Procédé suivant la revendication 11, dans lequel l'étape de traitement comprend l'utilisation d'une puissance maximale de 0,006 Js⁻¹cm⁻³ à 1,2 Js⁻¹cm⁻³ (0,1 watt/inch³ à 20 watts/inch³).

13. Procédé suivant la revendication 11, dans lequel l'étape de traitement comprend l'utilisation d'une puissance maximale de 0,006 Js⁻¹cm⁻³ à 0,6 Js⁻¹cm⁻³ (0,1 watt/inch³ à 10 watts/inch³).

14. Procédé suivant l'une quelconque des revendications précédentes, dans lequel la couche de polymère parylène a une teneur en impuretés zinc d'au plus environ 66 parties par milliard.

15. Procédé suivant l'une quelconque des revendications précédentes, qui comprend les étapes consistant à vaporiser un dimère de parylène et à pyrolyser le dimère de parylène pour former le monomère.

16. Procédé suivant la revendication 15, dans lequel l'étape de dépôt est mise en oeuvre dans une zone de dépôt (48) d'une chambre à vide (40).

17. Procédé suivant la revendication 15, dans lequel l'étape de pyrolyse est mise en oeuvre à l'extérieur de la zone de dépôt (48) de la chambre à vide (40).

18. Procédé suivant l'une quelconque des revendications 15 à 17, comprenant en outre l'étape consistant à introduire le monomère dans la zone de dépôt (48) de la chambre à vide (40).

19. Procédé suivant l'une quelconque des revendications 15 à 18, dans lequel l'étape de polymérisation comprend la polymérisation du monomère pour former un film de polymère parylène ayant une teneur en impuretés consistant en zinc d'environ 60 parties par milliard.

20. Structure à plusieurs niveaux, comprenant :
une première couche (12) ayant une surface ; et
une couche de polymère parylène (14) ayant des première et seconde surfaces, la première surface de la couche de polymère parylène étant opposée à la seconde surface de la couche de polymère parylène, la première surface de la couche de polymère parylène étant déposée le long de la surface de la première couche, la couche de polymère parylène étant formée à partir d'une matière de structure : dans laquelle
m a la valeur 0, 1, 2, 3 ou 4,
z est supérieur à 1,
G représente un atome d'halogène, un groupe alkyle, un groupe hydrocarboné cyclique, un groupe alkylène ou un groupe alkylyne de formule générale CnHyXw dans laquelle x représente un atome d'halogène, n est supérieur à zéro et la somme de y et w est au plus égale à 2n + 1,
**caractérisée en ce que** la couche de polymère parylène a une teneur en impuretés consistant en zinc d'au plus environ 66 parties par milliard et en ce qu'une couche de matière activatrice d'adhérence (16, 18) ayant une première surface et une seconde surface est présente, la première surface de la couche de matière activatrice d'adhérence étant disposée le long de la seconde surface de la couche de polymère parylène.

21. Structure à plusieurs niveaux suivant la revendication 20, dans laquelle la matière activatrice d'adhérence est choisie dans le groupe consistant en des organosilanes, des métaux, des oxydes métalliques, des oxydes de silicium et des oxydes semiconducteurs.

22. Structure - à plusieurs niveaux suivant la revendication 20 ou la revendication 21, comprenant en outre une seconde couche d'une matière activatrice d'adhérence placée de telle sorte que la couche de polymère parylène soit disposée entre les première et seconde couches de la matière activatrice d'adhérence.

23. Structure à plusieurs niveaux suivant la revendication 22, dans laquelle la première couche d'adhérence est constituée d'une matière électriquement conductrice.

24. Structure à plusieurs niveaux suivant la revendication 22, dans laquelle la seconde couche d'adhérence est formée d'une matière électriquement conductrice.

25. Structure à plusieurs niveaux suivant l'une quelconque des revendications 20 à 24, dans laquelle la couche de polymère parylène a une constante diélectrique d'au plus environ 2,6.

26. Structure à plusieurs niveaux suivant l'une quelconque des revendications 20 à 25, dans laquelle le polymère parylène comprend en outre une entité métallique.
